

Jan. 15, 1924.

1,480,675

J. F. DIRZUWEIT

ELECTRIC RESISTER AND ITS PROCESS OF MANUFACTURE

Filed Nov. 11, 1920



John F. Dirzuweit INVENTOR.

BY  
William W. Farney  
ATTORNEYS.

## UNITED STATES PATENT OFFICE.

JOHN F. DIRZUWEIT, OF LAUREL, MARYLAND, ASSIGNOR OF ONE-HALF TO WILLIAM W. VARNEY, OF BALTIMORE, MARYLAND.

## ELECTRIC RESISTOR AND ITS PROCESS OF MANUFACTURE.

Application filed November 11, 1920. Serial No. 423,232.

To all whom it may concern:

Be it known that I, JOHN F. DIRZUWEIT, a citizen of the United States, residing at Laurel, in the county of Prince Georges and 5 State of Maryland, have invented a certain new and useful Improvement in Electric Resistors and Their Process of Manufacture, of which the following is a specification, reference being had to the accompanying drawings, forming a part hereof.

My invention relates to electric resistors and especially to the method of their construction and treatment.

It has been the custom heretofore to construct resistors of irregular pieces of broken carbon or graphite, or to use continuous rods of carbon or other material. Resistors are also constructed of regularly shaped blocks or discs, which by reason of their high contact resistance lend themselves especially well for the construction of a mechanically strong element.

One of the chief disadvantages of all of the above named resistor elements is their 25 rapid disintegration at even moderate temperatures when in contact with oxygen. To obviate this especially in their use in the electric furnace, attempts have been made to prevent disintegration by operating such resistors in an atmosphere of producer gas, by introducing such gas into the melting chamber. This method, while exercising a beneficial action is impractical, as it is necessary to open the furnace frequently for 30 charging and pouring and if the internal pressure of the furnace is below atmospheric pressure, air will enter the furnace and will form an explosive mixture causing serious 35 accidents to life and property.

Attempts have also been made to protect resistors against the detrimental effects of the contained oxygen by surrounding them with a layer of silicon carbide, but such resistors are not practical for metallurgical 40 electric furnaces, where close temperature regulations are required.

It is known in the art that when a carbon filament is heated to incandescence in a hydro-carbon atmosphere, that any irregularities in the shape of the filament are automatically equalized, as at temperature above 50 3000 degrees F. the hydro-carbon gas breaks down and the free carbon combines with the

hottest part of the filament where the temperature is the highest.

It is also known in the art that carbon or any carbonaceous material when in contact with silica will absorb the silica, and at certain high temperatures form silicon-carbide. This silicon-carbide is not easily attacked by 60 oxygen, and if the penetration of the silica has reached sufficient depth, carbon may be made immune to oxygen provided the temperature does not reach the volatilization point of carbon.

The object of my invention in view of the above, is the construction of a resistor element for electric melting and heating furnaces, which will be mechanically strong, susceptible to close temperature regulation, 70 and which will not suffer from the detrimental effects of oxygen.

Referring to the drawings: Figure 1, represents in a longitudinal section part of a heating furnace provided with one or more 75 of my resistor elements; Fig. 2, shows an end elevation of my resistor element; Figs. 3 and 4 show side and end elevations of electric furnaces comprising several such resistor elements.

Similar numerals refer to similar parts throughout the several views.

1 and 2 are solid carbon or graphite electrodes which serve as current conductors to blocks or discs 3 composed of carbonaceous material. The number of these discs may be varied to suit different potentials. The electrodes 1 and 2 terminate in metallic electrode holders 8 and 9 and which are water cooled by water chambers 26.

Surrounding the complete electrode or resistor is a high refractory tube 5 terminating also in the metallic electrode holders 8 and 9. This tube may be made of any suitable material such as alundum, or silicon carbide.

The space between the refractory tube 5 and the carbon resistor is filled with pure silica sand 3 and is tightly packed. Electrodes 1 and 2 are fitted with metallic screw caps 6 and 7 slidably located in recesses to allow hand wheels 12 and 13 to exert pressure upon discs 3 to increase or decrease the resistance of the contact surfaces. Yokes 10 and 11 are supports for hand screws 12 and 13. Pipe 14 provides means for intro-

ducing any kind of inert or reducing gas into the space filled with silica sand and pipe 15 carries a pilot burner 24 indicating when the oxygen is expelled and the element is surrounded by such gas.

When the electric furnace is to be started, the above gas (say illuminating gas) is allowed to flow through the space filled with silica sand surrounding the resistor element 20 until all of the oxygen is expelled.

From the above it will be seen that by the operation of the furnace at high temperatures my improved resistors are made in place. I prevent the oxygen of the atmosphere from combining with the carbon by impregnating or case hardening the carbon or graphite electrode with silica or silicic acid. The process of doing the above is as follows:

20 The electrodes to be treated are packed with pure silica preferably of a size to pass through a number 20 mesh screen. Each electrode must be thoroughly covered. The ends of the electrodes are connected to current carrying electrodes of low potential. By passing electric current through the electrodes and resistors, heat is generated and when a temperature of 3400 degrees F. is reached the silica surrounding each electrode 25 or resistor is decomposed and is absorbed by the carbon or graphite electrodes or resistors. The penetration of the silica into the surface of the electrodes is a matter of time and can be controlled accordingly.

35 The properties acquired by the electrodes or resistors through the absorption of silica are very remarkable and make this material very desirable for the use of heating elements for electric furnaces. From practical experience it has been found that these electrodes or resistors will stand up to temperatures of 3400 degrees F. without any protection and can be exposed at that temperature to the atmospheric oxygen without 40 being affected.

This process will also increase the mechanical strength of the electrodes thereby reducing losses through breakage.

All kinds of shapes of electrodes may be 50 treated and made by this process and I do not limit myself to any shape.

After the furnace has been working for some time in actual use, to properly case 55 harden my resistors, the casing 5 and the surrounding silica may be destroyed or re-

moved without affecting the usefulness of my resistor.

Having thus described my invention, what I claim and desire to secure by Letters Patent is—

1. The process of forming electric resistors consisting of passing an electric current through a resisting material susceptible of combining with a surrounding medium at a high temperature while surrounded by a substance susceptible at high temperature of entering into combination with said resisting material.

2. The process of forming resistors consisting of a plurality of carbon sections aggregated, heating the aggregation to a sufficient temperature to cause the same to combine with silica supplied in a proper atmosphere in proximity thereto.

3. The process of forming resistors consisting of a plurality of carbon sections aggregated, heating the aggregation to a sufficient temperature to cause the same to combine with silica supplied in a proper atmosphere in proximity thereto consisting of a 75 hydrocarbon gas.

4. A resistor comprising a resisting material consisting of carbon blocks piled together, silica surrounding said pile and means of passing a gas through said silica.

5. A resistor comprising a resisting material consisting of carbon blocks piled together, silica surrounding said blocks means of passing a gas through said silica, terminals to said resistor provided with means of 80 cooling and means of conducting said gas.

6. A resistor comprising a resisting material consisting of carbon blocks piled together, silica surrounding said pile and means of passing a gas through said silica 95 and means of compressing said resisting material.

7. An electric resistor provided with water cooled terminals and regulating means between said terminals for compressing the 100 resistor, a conductor between said terminals comprising a pile of carbon blocks surrounded by silica contained in a refractory casing and means of introducing a gas through said silica from the exterior of said 105 terminals.

JOHN F. DIRZUWEIT.

Witnesses:

RICHARD P. HUTCHINS,  
WILLIAM W. VARNEY.